

## UNITED STATES PATENT OFFICE

2,506,040

## PROCESS FOR OBTAINING TRANSPARENT EFFECTS ON REGENERATED CELLULOSE FIBERS

Paul Walter Steinlin, Basel, Switzerland, assignor to Aktiengesellschaft Cilander, Herisau, Switzerland

No Drawing. Application July 31, 1946, Serial No. 687,507. In Switzerland April 22, 1943

5 Claims. (Cl. 8—118)

1

The present application is in the nature of a continuation in part of my earlier copending application Serial No. 533,788, filed May 2, 1944, now abandoned.

Transparent fabrics, also known as organdies, have as a rule been made from pure cotton materials, in particular muslin, or, more rarely, voile or other fine fabrics, such as cambric, etc. Organdies of especially fine quality were made of natural silk.

The process hereafter described relates to the production of plain or patterned, smooth or crepe transparent fabrics from materials consisting of staple fibre made from regenerated cellulose alone or of staple made from regenerated cellulose fibre and cotton, or of mixed cotton and staple fibre made from regenerated cellulose.

Various experiments were made in the past to transform textiles of this kind by the ordinary methods used for cotton fabrics. However, even by varying and adapting working conditions, such as concentration of acids and alkaline swelling agents, and the duration of the procedure, it proved impossible to turn out marketable goods. Indeed the materials hitherto produced were horny, brittle and stiffened, and in no way suited for practical use. The present process, on the contrary, produces transparent fabrics which perfectly satisfy all requirements as to appearance, lustre, softness and durability, and show a high degree of transparency combined with a remarkable clearness of weave.

By hot alkali is understood a treatment according to the present process with hot alkali solution of mercerizing strength, at a temperature of 25° C. or over, having a duration of 5 seconds or more.

These effects are obtained by subjecting the fabric, eventually after preparatory or supplementary treatment with swelling agents, to the action of strong alkali at room temperature for a short time and thereafter to the action of strong alkali at higher temperature.

The process is suited for fabrics made of pure staple fibre made from regenerated cellulose, or woven with cotton and staple fibre made from regenerated cellulose, and also for those woven with mixed staple fibre made from regenerated cellulose and cotton yarn. Naturally materials in which any or all of the above combinations are present, either in plain or pattern weave, including of course applications with embroidery or Swiss dotted weave, can also be treated by my process.

It is advantageous to delubricate and bleach

2

the fabric to be processed. Crude fabrics can, however, be treated in the same way. In this connection it should be borne in mind that, according to the invention, this process is suitable for use in any phase of pre-treatment.

My process can be used to advantage in combination with treatment by swelling agents. The order and manner in which these treatments are applied depend on the result desired.

- 10 By "treatment with strong alkali at room temperature" is understood a mercerizing treatment with alkali of at least 15° Bé. at temperatures ranging from —5° to +25° C. for a duration of 5 seconds or more.
- 15 Between the two successive alkaline treatments the fabric may be rinsed and neutralized. Nevertheless, it is not necessary to carry out one or both of these measures. By interposing rinsing or neutralization different results are obtained.
- 20 It is also possible to dry the fabric between the two alkaline treatments, or to leave it wet. These two procedures also lead to different results.

Patterned as well as plain transparent fabrics can be obtained with the present process by applying suitable reserves before the swelling treatment. For example imago effects can be achieved by printing with pigments, resulting in opaque non-transparent patterns. By this method it is possible, according to the type of process chosen, to use pigment carriers proof against acid and alkaline swelling agents, such as gums or artificial resins, which result in local opaque effects, or non-acidproof thickening agents which produce stiffened transparent designs in which the effect of contrast is due to the pigmentation alone. It is moreover possible to introduce reserves during any phase of the transforming process so as to achieve, for example, a transparent effect and then, by rinsing and subsequent swelling and shrinking, obtain the appearance of crepe. It is also possible to get intermediary effects by the imprint of swelling agents and subsequent treatment with hot alkali.

The reserves can even be applied during various phases of the process in such a way that the transformed material shows untreated and swollen, that is shrunken and transparent areas one next to the other.

It is evident that by printing in colours or by the use of coloured reserves such effects can be obtained in various tints.

Fabrics submitted to the present process can be dyed either before or after treatment. In this way, according to the method of procedure, the most varied results can be obtained, such as

plain transparent, or, according to the different affinity for the dye caused by different local treatment, shaded effects.

My process may be illustrated by means of a single example:

A fabric made from regenerated cellulose staple fibre is singed, bleached and tentered. It is then treated with NaOH of 30° Bé. at 20° C. for 10 seconds. After being rinsed and neutralized it is subjected to a further treatment with NaOH of 30° Bé. at 45° C., after which it is rinsed and neutralized and if required can be bleached, dyed or blued, according to the special effect desired.

I claim:

1. A multiple step process for obtaining transparent effects on a fabric consisting predominantly of regenerated cellulose staple fibre comprising a first step of treating said fabric with caustic soda of the order of 30° Baumé at a temperature of -5° to 25° C. for a period of time of the order of 5 to 10 seconds and a second step comprising treating said material with caustic soda of the order of 30° Baumé at a temperature of the order of 45° C. for a period of time of the order of 5 seconds.

2. A multiple step process for obtaining transparent effects on a fabric consisting predominantly of regenerated cellulose staple fibre comprising a first step of treating said fabric with caustic soda of the order of 30° Baumé at a temperature of the order of 20° C. for a period of time of the order of 10 seconds and a second step comprising treating said material with caustic soda of the order of 30° Baumé at a temperature of the order of 45° C. for a period of time of the order of 5 seconds.

3. A multiple step process for obtaining transparent effects on a fabric consisting predominantly of regenerated cellulose staple fibres comprising a first step of treating said fabric with caustic soda of mercerizing strength at temperatures of the order of -5° to 25° C. for a period of time of the order of 5 to 10 seconds, and a second step of treating said fabric with caustic soda of mercerizing strength at a temperature of the order of 45° C. for a period of time of the

order of at least 5 seconds but not substantially more than 5 seconds.

4. A multiple step process for obtaining transparent effects on a fabric consisting predominantly of regenerated cellulose staple fibres comprising a first step of treating said fabric with caustic soda of mercerizing strength at a temperature of -5° to 25° C. for a period of time of the order of 5 to 10 seconds and neutralizing and rinsing the fabric, and a second step of treating the fabric with hot caustic soda of mercerizing strength at a temperature of the order of 45° C. for a period of time of the order of at least 5 seconds but not substantially more than 5 seconds.

5. A multiple step process for obtaining transparent effects on a fabric consisting predominantly of regenerated cellulose staple fibres comprising a first step of treating said fabric with caustic soda of mercerizing strength at a temperature of -5° to 25° C. for a period of time of the order of 5 to 10 seconds and rinsing and drying said fabric, and a second step of treating the fabric with hot caustic soda of mercerizing strength at a temperature of the order of 45° C. for a period of time of the order of at least 5 seconds but not substantially more than 5 seconds.

PAUL WALTER STEINLIN.

#### REFERENCES CITED

The following references are of record in the file of this patent:

#### UNITED STATES PATENTS

| Number       | Name          | Date          |
|--------------|---------------|---------------|
| 1,439,517    | Heberlein     | Dec. 19, 1922 |
| 1,922,308    | Lilienfeld    | Aug. 15, 1933 |
| 1,989,100    | Lilienfeld    | Jan. 29, 1935 |
| 40 1,998,576 | Heberlein     | Apr. 23, 1935 |
| 2,202,200    | Haller et al. | May 28, 1940  |

#### FOREIGN PATENTS

| Number     | Country       | Date         |
|------------|---------------|--------------|
| 45 273,327 | Great Britain | Aug. 9, 1928 |
| 323,175    | Great Britain | Jan. 2, 1930 |